

H. W. McQUAID.

PROCESS OF DETERMINING THE SUITABILITY OF STEEL FOR CASE HARDENING.  
APPLICATION FILED AUG. 1, 1921.

1,425,787.

Patented Aug. 15, 1922.



*Fig. 2.*



Inventor:  
Harry W. McQuaid,  
by *Samuel L. Cane*,  
his Attorney.

# UNITED STATES PATENT OFFICE.

HARRY W. MCQUAID, OF CANTON, OHIO, ASSIGNOR TO THE TIMKEN ROLLER BEARING COMPANY, OF CANTON, OHIO, A CORPORATION OF OHIO.

## PROCESS OF DETERMINING THE SUITABILITY OF STEEL FOR CASEHARDENING.

1,425,787.

Specification of Letters Patent. Patented Aug. 15, 1922.

Application filed August 1, 1921. Serial No. 488,885.

To all whom it may concern:

Be it known that I, HARRY W. MCQUAID, a citizen of the United States, and a resident of the city of Canton, in the county of Stark and State of Ohio, have invented a new and useful Improvement in Processes of Determining the Suitability of Steel for Casehardening, of which the following is a specification.

10 My invention relates to a method of testing steel to determine whether it is suitable for use in the manufacture of devices that require to be hardened. Heretofore it has been commonly assumed that the ability of 15 steel to react properly to the usual hardening treatment depended wholly upon its chemical composition and could be told in advance of the hardening operation by simple chemical analysis of the steel. I have discovered, 20 however, that traces of impurities too minute to be detected by ordinary chemical analysis may wholly unfit a steel for hardening; and it is the object of the present invention to devise a reliable method of determining 25 whether steel of a particular lot is suitable for hardening. It consists principally in carburizing a sample of such steel and microscopically examining the same as hereinafter specified.

30 In the accompanying drawing, which forms part of this specification, and wherein like reference letters refer to like parts wherever they occur,

Fig. 1 is a diagrammatic view illustrating 35 the characteristic appearance, under high magnification, of a polished and etched section through the hypereutectoid zone of a "normal" steel that has been carburized and slowly cooled; and

40 Fig. 2 is a similar diagrammatic view illustrating the characteristic appearance, under high magnification, of a polished and etched section through the hypereutectoid zone of an "abnormal" steel that has been 45 carburized and slowly cooled.

In the accompanying drawing, the reference letter C indicates areas of cementite ( $Fe_3C$ ) sometimes called iron carbide. The reference letter P indicates pearlitic areas 50 or areas of pearlite. The reference letter F indicates areas of ferrite.

In carrying out my process, I take a suitable sample of steel that is to be tested.

This sample is then carburized in any suitable manner; for instance, it is packed in 55 suitable carbonizing material and gradually raised to a suitable carburizing temperature, say about 1700 degrees Fahrenheit. This carburizing temperature is usually reached in about ten or twelve hours, after which the 60 sample is allowed to cool gradually.

A section is then made of the sample and the hypereutectoid zone of such section is carefully polished and etched in a well known manner with some suitable etching fluid 65 such as picric or nitric acid solution. The polished and etched surface of the metal is then examined under a microscope of sufficient magnification to clearly show the micro-structure of the section, say magnification of from fifty to two hundred diameters.

I have discovered that when two steels of apparently the same chemical composition, one of which is suitable for hardening (and 75 which is herein referred to as the "normal" steel) and the other of which is not suitable for hardening (and which is hereinafter referred to as "abnormal" steel), are case-carburized and slowly cooled and sections made 80 through the hypereutectic zone of their cases and suitably prepared for microscopic examination, there is a characteristic difference in their appearance. The etched normal sample shows large grains of pearlite separated by fine lines of cementite, so that the structure appears to be that of large grains of lamellar structure separated by fine lines of cementite. On the other hand, in the sample that is unfit for hardening, the grains 85

are smaller in size and less uniform in appearance and the ridges of cementite are more numerous than in the normal sample. Evidence of the tendency of the pearlite areas to form free cementite on a background of ferrite is apparent. Presumably, 90 the difference in the structure of the normal steel and of the abnormal steel is due to non-metallic impurities present in quantity usually too small to be easily noted by 100 chemical analysis. My researches indicate that this is clearly the case where the impurity is present in the form of oxide, which impurity is liable to be introduced during the furnace operation and which is 105 insufficiently eliminated by the use of deoxi-

dizing agents and which remain present in such minute quantity as to defy ordinary chemical analysis.

The compounds of other non-metallic elements, as well as those of oxygen, are segregated in minute particles that are distributed through the steel without being dissolved therein, and, under microscopic examination, such particles are clearly differentiated from the steel and present characteristic appearances by which they may be identified generically or specifically.

In determining microscopically whether or not the steel is "normal" or "abnormal" it should be noted that the hypereutectoid zone is necessary to develop the breaking down of the pearlite and while the gradation zone of the abnormal steel can easily be distinguished from the gradation zone of normal steel after carburizing, the eutectoid zone shows little difference, the pearlite in the abnormal steel apparently having a slight tendency to become coarsely lamellar. The presence of cementite, however, apparently facilitates the breaking down of the pearlite and hence the higher the carbon concentration, i. e. the greater the amount of excess cementite, the more complete will be the breaking down of the pearlite. Therefore, carburizing compounds which produce a very high carbon case will indicate more clearly whether or not the steel is "normal" or "abnormal."

Annexed hereto are typical microphotographs of the hypereutectoid zones of normal and abnormal steels after case-hardening and slow cooling, the magnification in each case being two hundred diameters. In photograph No. 1, which shows the normal steel, the pearlite is very finely lamellar and the cementite exists as well defined lines of fine but continuous formation at the boundaries of the crystals. In photograph No. 2, which shows the abnormal steel carburized and cooled under the same conditions as the normal steel of photograph No. 1, the pearlite is broken down into the form of massive cementite and free ferrite, the cementite appearing as ridges on a white background of ferrite. While there will be differences in detail in photographs of normal steels, the appearance shown in photograph No. 1 is characteristic; and likewise, the appearance typical or characteristic of an abnormal steel is represented in photograph No. 2, although individual photographs will differ in detail.

For the purpose of completing, studying and recording tests, microphotographs may be made of suitably polished and etched sections of carburized samples. By study and comparison of such photomicrographs of normal and abnormal samples, one soon learns to recognize the appearances that characterize steel as fit or unfit for harden-

ing purposes; and photomicrographs of such samples may be preserved for purposes of record or study.

While the principal object of the invention is to be able to determine from a carburized sample the suitability of a given lot of steel for properly reacting to hardening treatment, it is noted that the carburized sample is not hardened, for the rapid quenching required for hardening produces a very different appearance from that of slow cooling. Likewise, as the characteristic appearance of "abnormal" steel is due to the presence of impurities therein and as such impurities affect the quality of the steel for other uses than hardening, the process above described is applicable to other purposes than simply determining the suitability of steel for hardening.

What I claim is:

1. The process of determining the suitability of steel for hardening which consists in carburizing a sample thereof and microscopically examining a section of said sample through its carburized case.

2. The process of determining the suitability of steel for hardening which consists in case-carburizing and slowly cooling a sample thereof, preparing a section of the carburized case for microscopic examination, and microscopically examining such section.

3. The process of determining the suitability of steel for hardening which consists in case-carburizing and slowly cooling a sample thereof, preparing a section of the carburized case for microscopic examination, and microscopically comparing such section with a similarly treated sample of steel of known standard qualities.

4. The process of determining the suitability of steel for case-hardening which consists in case-carburizing and slowly cooling a sample thereof, and preparing and microscopically examining a section of said sample through the hypereutectoid zone of its carburized case.

5. The process of determining the suitability of steel for case-hardening which consists in case-carburizing and slowly cooling a sample thereof, making a microphotograph of a section of said sample through the hypereutectoid zone of the carburized case and comparing the same with a like photograph of a steel of known quality.

6. The process which consists in case-carburizing and slowly cooling a sample of steel, making a microphotograph of a section of said sample through the hypereutectoid zone of the carburized case and comparing the same with a like photograph of a steel of known quality.

7. The process of determining the suitability of steel for case-hardening which consists in case-carburizing and slowly cool-

ing a sample of steel, polishing and etching a section of said sample through the hypereutectoid zone, making a microphotograph of such section and comparing the same with a like photograph of a steel of known quality.

5 8. The process which consists in case-carburizing and slowly cooling a sample

of steel, polishing and etching a section of said sample through the hypereutectoid 10 zone, making a microphotograph of such section and comparing the same with a like photograph of a steel of known quality.

Signed at Canton, Ohio, this 20th day of July, 1921.

HARRY W. McQUAID.